

Oct. 18, 1955

W. F. HIGGINS ET AL

2,721,172

CONSUMABLE METAL ANODES

Filed July 5, 1951

FIG. 1.



FIG. 2.



FIG. 3.



*Inventor*

William Frederick Higgins &  
William Godfrey Waite

By *Theodore H. Higgin*,  
Attorney

## 1

2,721,172

## CONSUMABLE METAL ANODES

William F. Higgins, Salford, and William Godfrey Waite, Piccadilly, London, England, assignors to F. A. A. Hughes & Co. Limited, London, England, a British company

Application July 5, 1951, Serial No. 235,214

Claims priority, application Great Britain July 12, 1950

2 Claims. (Cl. 204—197)

This invention relates to an improved construction for consumable metal anodes used in the galvanic protection of corrodible metal structures.

In the galvanic protection of buried metallic structures or structures immersed in an aqueous solution, consumable electrodes of a metal anodic to the metal of the structure are buried in the earth or immersed in the water near the structure and are connected thereto by electrical conductors. The resulting flow of current maintains the structure cathodic with respect to the soil or water and greatly arrests the corrosion. The consumable anodes hitherto used have consisted of blocks of strongly basic metal such as zinc or magnesium or base alloys of these metals with a plain surface which is intended to be consumed at a fairly even rate. Such anodes whilst effective, maintain a fairly constant current output throughout most of their lives.

It is common experience that the current generated is in certain cases greater than that required for adequate protection, and the rate of usage of the anode is consequently higher than is desirable. This is especially the case in sea water where the electrolytic resistance may be very low. In such circumstances the anode has a shorter life than might otherwise be the case.

It is possible to limit the current actually applied to the structure to be protected by means of suitable electric resistances inserted in the metallic circuit, but this is not an ideal method since it tends to reduce the useful current without materially affecting the rate of chemical reaction on the anode surface which gives rise to the current. Thus the use of resistances is a wasteful process.

The current generated by the anode is a function, among other factors, of the surface area of the anode exposed to the electrolyte and taking part in the chemical process resulting from contact of the anode with the electrolyte.

One obvious way of limiting the current, is to use anodes of small superficial area, but this method largely defeats its object since such small anodes would necessarily have a short life and would require to be replaced at unduly short intervals.

According to the present invention the current is controlled at the place of origin, that is, the interface between anode and electrolyte, by providing a coating on its surface which partly shields the anode surface from the electrolyte thereby reducing the rate of reaction of the anode with the electrolyte, said coating being made of a material which is substantially unattacked by the electrolyte.

The shielding means may be such that only a portion of the anode surface is exposed to reaction with the electrolyte at any time; or, alternatively such that all the surface, or substantially all the surface, is exposed, but in such a way that the access of electrolyte is restricted and the rate of current generation consequently reduced; or by a combination of both these methods.

It is possible by this arrangement to use a large anode containing a volume of material sufficient for long con-

## 2

tinued protection and to ensure long continued protection by exposing the material of the anode regularly and progressively to the electrolyte. It will be shown later that it is possible also by a slight variation in technique at the time of installing the anode, to secure an initial high rate followed, after a due period, by a smaller regular rate, a method which is often of considerable value in the art of galvanic protection.

In carrying the invention into effect the anode, (which may be of any convenient metal or alloy known to be suitable for the purpose of supplying galvanic current) according to one example, may be cast or wrought as a solid cylinder or bar, having a galvanised steel or other metal connection provided at one end. This connection is for the purpose of coupling the anode to the structure to be protected. This connection however is preferably not located deeply within the length of the anode but is confined to one end. The anode body itself, including the end bearing the connection, is sheathed in impervious and electrically insulating material with the exception of one area, conveniently, but not necessarily, the end remote from the connector. Thus the extreme end only of the anode is, in this case, presented to the electrolyte, and as the area of this end can be made much smaller than the total area of the anode, and in any desired proportion thereto, the current generated will be smaller in like proportion. Thus the operation of the anode is restricted so that it is consumed from the end only, and as the surface is used up in the reaction fresh metal is exposed progressively throughout the length of the anode until it is entirely consumed.

In experiments we have made, a cylindrical anode was constructed on the above described principle, of such dimensions that the area of the exposed end was one-tenth of the total area. On immersion in sea water the current generated was found to be approximately one-tenth of that generated by an identical anode in which the whole of the body was exposed. Consumption of the totally exposed anode was uniform over the whole surface, while that of the shrouded anode took place only on the exposed end and progressed steadily up the containing tube formed by the shroud. Since the two identical steel sheets to which the two anodes were severally coupled remained quite bright and free from corrosion it is obvious that the smaller current delivered by the shrouded anode was sufficient for galvanic protection of the steel and that the ten times larger current delivered by the unshrouded anode was abnormally wasteful.

If desired the shrouding of the anodes may be carried out in such a way that the impervious wrapping can be readily stripped back from the surface to any degree desired, thus enabling the user to commence protection with a greater surface (and therefore a proportionately higher current) than would be obtained from the exposed end surface alone; later, when the uncovered length has been consumed, the end surface only will remain exposed, generating current at a rate proportional to its area. Thus the advantage will be secured of high initial current where desired, coupled with long life at a lower subsequent rate.

In the form of the invention described above the sheathing material is designed to remain in situ as the anode is consumed, so that access of the electrolyte to the end surface becomes gradually more restricted as the surface retreats down the tube. This is of no practical consequence because the diameter of the anode is so chosen that the restriction of circulation of fresh electrolyte down the gradually increasing length of sheathing tube is negligible.

In another form of the invention the sheathing takes

the form of an impervious but somewhat friable material, sufficiently strong to withstand handling when containing the anode, but capable of being gradually broken away by the increasing volume of the corrosion product of the anode and the action of sea water, as the anode is dissolved away. In this form of the device the reactive end of the anode is always presented to the electrolyte completely unrestricted. A suitable material for the purpose intended can be produced from bitumen or bitumen-like compounds incorporating a proportion of 10 fillers such as powdered slate or stone.

In another form of the invention, instead of a more or less completely impervious sheath, an elastic membrane is used, designed to be of a semipermeable or microporous nature. In this case it may be applied over the whole surface of the anode and limits the access of electrolyte by virtue of, and in proportion to, its permeability. The elastic nature of the sheath provides for the increased volume due to the corrosion product of the anode through its reaction with the electrolyte. For this purpose sheaths of microporous rubber may be used, or the same effect may be achieved by the application of certain paint films.

According to a still further form of the invention the anode is provided with a sheath of a metal or alloy more noble than the metal or alloy of which the anode is made. For example the sheath may be made of aluminium or aluminium base alloy which may be of foil thickness or may have a thickness up to say one quarter of an inch. If desired an aluminium tube may have a molten magnesium alloy poured into it to form the sheathed anode. We have found that a magnesium anode sheathed with aluminium or aluminium alloy with a metal to metal contact between the magnesium alloy and the aluminium or aluminium alloy gives satisfactory results. If desired however an electrically insulating coating e. g. of bitumen may be disposed between the two metals.

The invention is illustrated by way of example in the accompanying diagrammatic drawings wherein:

Figure 1 is a perspective view of an anode made in accordance with the invention;

Figure 2 is an underneath plan view thereof;

Figure 3 is a perspective view of a modified form of the anode.

In the construction shown in Figures 1 and 2, the anode

15 consists of a cylindrical block 10 of magnesium base alloy having a steel rod 11 cast into its top end, and having a tubular coating 12 of aluminium having a top wall 13 which encloses the upper surface of the block 10, this wall 13 having a central hole through which the rod 11 passes. This tube can be inverted and the said central hole closed by a sand mould while the molten magnesium is poured into it. The finished anode thus has the lower circular end surface of the magnesium alloy uncovered and this is the only area subject to the electrolytic action. As shown in Figure 3 the magnesium alloy may extend below the lower end of the aluminium coating so that a larger area is initially exposed to electrolytic attack which is sometimes desirable in order to provide a larger current during an initial period until polarisation is effected whereafter a smaller current is desired. After the lower projecting end of the magnesium alloy has been consumed, only the circular lower surface is subject to attack.

20 We claim:

1. A consumable metal anode for the galvanic protection of metal structures comprising an anode block made essentially of magnesium or magnesium base alloys, a ferrous metal rod having one end embedded in one 25 end of said block and extending outwardly therefrom, a protective sheath surrounding and contacting the outer surface of said block and covering the end face from which the rod extends, the other end of the block being left free of the sheath, said sheath being made essentially of more noble aluminum or aluminum base alloys to reduce the rate of reaction of the anode with the electrolyte.

2. A consumable metal anode for galvanic protection of metal structures as defined in claim 1 and said anode being free of the sheath for a small part of the outer 35 surface adjacent to and immediately above the end face which is already free of the sheath.

#### References Cited in the file of this patent

#### UNITED STATES PATENTS

|           |              |               |
|-----------|--------------|---------------|
| 685,176   | Ross         | Oct. 22, 1901 |
| 1,506,306 | Kirkaldy     | Aug. 26, 1924 |
| 2,157,180 | Little       | May 9, 1939   |
| 2,459,123 | Bates et al. | Jan. 11, 1949 |
| 2,489,739 | Bialosky     | Nov. 29, 1949 |
| 2,541,062 | Hoxeng       | Feb. 13, 1951 |